

Nov. 8, 1932.

N. SLATER

1,887,477

PILE FABRIC

Filed Jan. 12, 1929

Fig. 1.



Fig. 2.



Inventor  
Nelson Slater

By his Attorneys  
Hoguet & Meany

## UNITED STATES PATENT OFFICE

NELSON SLATER, OF WEBSTER, MASSACHUSETTS, ASSIGNOR TO S. SLATER & SONS, INC.,  
OF WEBSTER, MASSACHUSETTS, A CORPORATION OF MASSACHUSETTS

## PILE FABRIC

Application filed January 12, 1929. Serial No. 332,090.

This invention relates to a pile fabric, and a method for making same.

It is an object of my invention to provide a novel type of pile fabric.

5 Another object is to provide a pile fabric, and a process for making same, in which certain steps usually necessary have been eliminated.

10 A further object is to provide a pile fabric with a more ornamental and durable pile surface than has heretofore been possible. Other objects will appear as the description proceeds.

15 It has long been known to coat a fabric with a layer of an adhesive, apply a layer of some fibrous material and then raise a nap by means of a wire brush, or otherwise. This, however, has certain disadvantages, such as the difficulty of raising the nap to exactly the 20 desired degree without detaching a large part of the fibers; the tendency of the fibers to lie flat, since they are applied flat and the consequent difficulty of maintaining a satisfactory nap; the fact that the layer of adhesive 25 is obvious to the eye, and masks to a certain extent the weave of the base fabric, thus making the finished product appear somewhat less like a fabric. All these disadvantages I have overcome, and are avoided in the fabric, 30 the making of which I shall presently describe.

35 My invention will be best understood by reference to the following description, taken in conjunction with the accompanying drawing, in which like reference characters represent like elements, and in which

40 Fig. 1 is a broken plan view, showing my completed fabric and the different component layers thereof, and

45 Fig. 2 is a section taken on line 2—2 of Fig. 1.

In the drawing I have indicated at 12 a base fabric. This can be of any desired material, such as duck, etc.; the material used in any given case being chosen with a view to its cheapness and durability.

50 At 10, I have indicated fibers, which are forced through the base fabric, with a short end 16 projecting downwardly, and a longer

portion, which is to form the pile or nap, projecting upwardly from said base fabric.

I may use fibers of any sort that I find desirable. Wool, hair, cotton, silk, rayon, etc., are all obviously suitable, used either alone or in combination.

55 In order to anchor the fibers, and prevent their becoming detached from the base fabric, I apply to the lower short ends, which are indicated at 16, a coating of a cementing material 14. Pyroxylin is a suitable material to use for this cement; although I obviously do not limit myself thereto. Latex, varnish, or any similar cementing substance may be 60 used equally well.

65 The advantages of my fabric are obvious. It is unnecessary to raise a pile, as must be done if the pile and the cement are on one side of the base fabric; mere brushing up will produce a pile effect that is quite desirable 70 and beautiful. There is much less tendency for the pile to flatten out, since its attachment is vertical to the base fabric, instead of parallel thereto. Compared with fabrics in which the fibers are merely needled through 75 the base fabric, the provision of a cement of course greatly increases the durability.

80 While I have spoken of a base fabric, it is clear that I could use other materials. Leather, rubber or composition bases of any type might be used, or even paper, if such should be found desirable.

85 Other changes might be made, such as are within the province of one skilled in the art. For example, the fibers might be inserted at an acute angle to the base member, instead of perpendicularly thereto, thus giving a novel effect. Such changes are to be considered as comprised and included in my invention, 90 which is to be limited only by the prior art and the scope of the appended claims.

95 In an attempt to produce a pile fabric of the general description and the structure which I have described, it has sometimes been the practice to lay a part of the material upon the base and force some of the bat material into the base and in fact, through it, so that the fabric projecting through it can be treated as pile, and the bat on the opposite side secured to the base by pyroxylin or 100

other waterproof cement. The method of producing such a pile is objectionable, first because it is not economical because of the fiber which would make good pile, being allowed to lie in a useless bat upon the base, and further because it has been found impractical to make as full and nice a layer of protruding pile as is desired. By my method, however, it will be seen that there is no bat and that the pile fibers are substantially all of them forced entirely through the base and that the shorter ends of the fibers on one side of the base are anchored in a suitable waterproof cement. In this way all the material which would otherwise lie in a bat is used and a thick, nice, pile is produced on the other side.

I claim:

1. An improved pile fabric comprising a base having a mass of pile fibers substantially all of which project entirely through it and with the protruding fibers on one side only anchored to the base by a waterproof cement.
2. An improved pile fabric comprising a base, and a mass of fibers substantially all of which project through said base so as to protrude on both sides thereof, said fibers being anchored to said base by a cement applied to one face thereof.
3. An improved pile fabric comprising a base, and a mass of fibers substantially all of which project through said base so as to protrude on both sides thereof, said fibers projecting further on one side than on the other and the shorter protruding ends being anchored to said base by means of a coating of cement.

In testimony whereof, I have signed my name to this specification this 11th day of January 1929.

NELSON SLATER.

45

50

55

60

65